

Patented Sept. 28, 1948

2,450,034

## UNITED STATES PATENT OFFICE

2,450,034

GROUNDWOOD BLEACHING BY  
HYDROSULFITEHoward J. Cronin, Glens Falls, N. Y., assignor to  
International Paper Company, New York, N. Y.,  
a corporation of New YorkNo Drawing. Application December 1, 1943,  
Serial No. 512,475

4 Claims. (Cl. 8—104)

1

It is an object of this invention to provide an improved bleaching process particularly applicable to the bleaching of ground wood pulp.

It is a further object of this invention to provide an improved bleaching process involving the use of reducing or deoxidizing agents.

It is a further object of this invention to provide a bleaching process involving the use of a reducing or deoxidizing agent in which the bleaching effect will be substantially stable and not subject to retrogression or degradation with lapse of time.

For the purpose of this disclosure a reducing agent may be defined as any compound which will remove or tend to remove oxygen from chemical combination at temperatures below the boiling point of water and which will do so while in contact with oxygen compounds in an aqueous solution or suspension.

Heretofore it has been axiomatic in the art that bleaching accomplished by the use of reducing or deoxidizing agents is subject to the defect of being transitory, that is, the material to be bleached attains a considerable bleaching effect during contact with the active ingredient but on subsequent exposure to air or even upon agitation or heating the material apparently reoxidizes, with a restoration of the original color and consequent elimination of the bleaching effect. This invention, while particularly applicable to the bleaching of ground wood pulp, is actually applicable to the bleaching of various materials and, except as explicitly limited in the subjoined claims, the process is deemed to be applicable to any material, whether a papermaking pulp or a textile-making fibre.

The term "efficiency of the process" as used herein relates to the cost of securing a given improvement of color and does not relate to the chemical efficiency of the reactions involved. A given increase in brightness is worth just so much money in saleability of the finished product. This sets a maximum limit upon the overall cost of producing the improvement. This overall cost is made up not only of the direct cost of the bleaching agent or agents and the direct cost of labor, but also of the depreciation of the equipment involved, the floor space and buildings occupied by such equipment, and the cost of pumping and agitating the mixtures. Accordingly, the optimum conditions from the standpoint of cost efficiency may or may not have any relation to the optimum conditions for chemical efficiency.

This disclosure deals primarily with bleaching obtained by the use of zinc or sodium hydrosul-

2

phite, but it is to be understood that any reducing agent compatible with the particular material to be bleached may be employed by the method herein set forth. This includes the hydrosulphites of various metals other than zinc or sodium, together with various bisulphites and other reducing compounds. The selection of a particular reducing agent will be governed, first, by consideration of its compatibility with the material to be bleached and, second, by considerations of cost, and such selection is considered to be within the skill of the ordinary "person skilled in the art." When certain materials are exposed to the action of certain reducing compounds there may take place "side reactions" which themselves will generate colored compounds detrimental to the desired bleaching effect. The determination of whether such reactions will take place as between any particular material to be bleached and any particular reducing agent is easily determinable by routine tests. It is not necessary to determine the nature or even the existence of such side reactions. It is only necessary to determine whether an economic quantity of reducing agent will produce, first a sufficient improvement in brightness, and second a substantially stable improvement.

The essence of this invention lies in intermixing the reducing agent and the material to be bleached with a minimum of agitation and, immediately upon completion of the mixing step, maintaining the mixture in a condition of quiescence for a substantial period of time. It has been determined that if a sufficient period of quiescence follows the step of intermixing carried out with minimum agitation, there results a bleaching effect which persists over considerable periods of time with slight, if any diminution.

The period during which the mixture of stock and bleaching agent should remain quiescent following the mixing step is largely dependent upon the color improvement desired and this in turn is, of course, dependent upon the brightness of the stock before the bleaching step. There will be a perceptible increase in brightness in as little as half an hour and the brightness will continue to increase measurably for as much as twenty-four hours. After five hours, however, the increase is relatively small and quite slowly attained, so that as a commercial proposition it will not usually be desirable to provide a period of quiescence longer than four to five hours. It has been determined that after four hours' quiescence the mixture may be violently agitated without substantial decrease in brightness, although if agitation be resorted to after much less than four

hours there will be a diminution in brightness. Since in the handling of papermaking stock violent agitation is necessarily involved in supplying the stock to the paper machine, diluting and running it over the wire, such steps should be deferred at least three hours from the conclusion of the mixing step.

In using zinc or sodium hydrosulphite it has been determined that the use of 1% of the hydrosulphite by weight as against the dry weight of the pulp to be bleached yields substantially better results than the use of  $\frac{1}{2}\%$ , but the use of  $1\frac{1}{2}\%$  contributes very little in the way of additional results over the use of 1%. Accordingly, the use of hydrosulphite in excess of 1% of dry weight of pulp is not recommended, although so far as the essence of this invention is concerned any proportion by weight may be used.

Utilizing from 1% to  $1\frac{1}{2}\%$  of hydrosulphite (based on the dry weight of the pulp) there is evidence to indicate that the activity of the hydrosulphite is substantially exhausted at the end of four hours of quiescence of the mixture, since the color improvement thereafter is slight and proceeds slowly. The precise chemistry of the reaction has not been determined and is considered immaterial to the present disclosure. The fact is that most of the improvement which can possibly be secured takes place within four to five hours' quiescence and that the least improvement which would justify the cost of the process is attained within approximately one hour.

The temperature at which the reaction takes place has an effect upon the ultimate effectiveness of the bleach and upon the duration of the period of quiescence. An increase in temperature from 70° F. to 80° seems to make little difference, but an increase to 100° F. increases the total improvement in brightness and shortens the time in which a given improvement occurs.

The consistency of the stock to be bleached is also a factor. Bleaching takes place in a water suspension of the stock and it has been found that dilution of the suspension below  $2\frac{1}{2}\%$  (dry weight of stock divided by total weight of the suspension) decreases the efficiency of the process, while an increase of consistency beyond 5% (similarly calculated) equally impairs the efficiency of the process. This impairment of the efficiency of the process by increasing the consistency beyond 5% is believed to be due to the fact that higher consistencies require a greater amount of agitation for thorough distribution of the bleaching agent. Theoretically, almost no agitation would be required at infinite dilution and therefore the efficiency of the process would be greatest at infinite dilution. The practical requirements of an operating plant, however, are responsible for setting 2% as minimum consistency. At such consistency the slurry will contain 39 tons of water for each ton of fibre whereas at 1% consistency there are 99 tons of water for 1 ton of fibre, and the problems of storage and pumping make such extreme dilutions uneconomical. It has also been determined that the best results are secured when the reducing agent in dry powdered form is mixed with the stock. However, a 10% solution of the bleaching agent may be preserved for a limited time (preferably not more than two or three hours) under conditions of mild agitation and may be used with satisfactory results. In practice, the convenience of using a solution in place of handling a dry powder will probably dictate the use of the liquid form of bleaching agent. In addi-

tion, less agitation is required for sufficient mixing in the case of a liquid than in the case of a dry powder.

It is to be noted that in the use of this invention optimum conditions are encountered as dilution increases. This is counter to the trend of development in all other bleaching processes which under modern practice can be carried on at greater concentrations.

Experiments have shown some improvement in color when the pulp is adjusted to pH 7 prior to addition of the hydrosulphite. However, such advantage is very slight and it is not considered to be commercially important to make such adjustment. In commercial operation with ground wood pulp fresh from the grinders and having a pH of approximately 5.5 the addition of the hydrosulphite lowers the pH to a range of 4.8 to 5.0. It has been found that entirely satisfactory results are secured within this range inasmuch as a permanent increase in brightness of at least 4 points is obtained in a period of three and one-half hours.

From the standpoint of cost efficiency the optimum conditions under which this process may be carried out are set forth in the following example:

- (1) Zinc hydrosulphite should be used in an amount equal to 1% of the dry weight of fibre to be bleached.
- (2) Temperature should be maintained at or slightly above 100° F.
- (3) The consistency of the suspension should be not less than  $2\frac{1}{2}\%$  nor more than 5%.
- (4) The hydrosulphite should be mixed with the suspension with the least possible agitation.
- (5) Following the mixing step the mixture should remain quiescent for not less than three and one-half hours, but it is not necessary or particularly advantageous to maintain it quiescent for more than four or five hours.

As another example the process may be carried out as above except that sodium hydrosulphite is used in the place of zinc hydrosulphite.

A specific example of the use of this process with ground wood pulp will now be given. Ground wood pulp having an initial brightness of 59.6 (on the G. E. brightness meter) at pH 5.6 and consistency of  $3\frac{1}{2}\%$  had added to it, with a minimum of agitation, zinc or sodium hydrosulphite in an amount equal to 1% of the dry weight of the pulp. The pH of the mixture dropped to 4.9. A temperature of approximately 100° F. was maintained and the mixture was allowed to remain quiescent for three and one-half hours. At the end of this period the brightness had risen to 63.7, showing a gain of 4.1 points over the original brightness. The bleached pulp was then formed into paper by usual processes and the brightness of the paper thus formed was 64. After a period of six weeks during which samples of the paper were stored in a desk drawer the brightness was 65.

In another commercial operation a freshly ground spruce pulp having an initial brightness of 66.6 was treated substantially as set forth in the preceding example and at the end of three hours the brightness had risen 6.3 points to 72.9. At the end of five hours the brightness had risen 0.3 points to 73.2. This example is illustrative of the relatively slight improvement in color which is attained by prolonging the period of quiescence substantially beyond three to three and one-half hours. It is also illustrative of the applicability of the present process to the bleaching of a

2,450,084

5

groundwood pulp of unusually high initial brightness.

The above detailed description and the specific examples herein set forth relate to preferred forms of the present invention. It is obvious that modifications and variations may be resorted to by those skilled in the art within the scope of the following claims:

I claim:

1. A method of bleaching an aqueous suspension of groundwood pulp comprising: adding zinc hydrosulphite in an amount equal to 1% of the dry weight of pulp; mixing said zinc hydrosulphite with said suspension with a minimum of agitation and thereafter maintaining said mixture quiescent for not less than three hours. 15

2. A method of bleaching groundwood pulp comprising: making an aqueous suspension of pulp of consistency not less than 2½% nor more than 5%; adding zinc hydrosulphite in an amount equal to not less than ½% nor more than 1½% of the dry weight of pulp; mixing said zinc hydrosulphite with said suspension with a minimum of agitation; and thereafter maintaining said mixture quiescent for not less than three nor more than five hours.

3. A method of bleaching an aqueous suspension of groundwood pulp comprising: adding zinc hydrosulphite in an amount equal to 1% of the dry weight of pulp; mixing said zinc hydrosulphite with said suspension with a minimum of agitation; thereafter maintaining said mixture quiescent for not less than three hours, and maintaining the temperature of said mixture at substantially 100° Fahrenheit throughout said period 35 of quiescence.

6

4. A method of bleaching groundwood pulp comprising: making an aqueous suspension of pulp of consistency not less than 2½% nor more than 5%; adding zinc hydrosulphite in an amount equal to not less than ½% nor more than 1½% of the dry weight of the pulp; mixing said zinc hydrosulphite with said suspension with a minimum of agitation; thereafter maintaining said mixture quiescent for not less than three nor more than five hours; and maintaining the temperature of said mixture at substantially 100° Fahrenheit throughout said period of quiescence.

HOWARD J. CRONIN.

#### REFERENCES CITED

The following references are of record in the file of this patent:

#### UNITED STATES PATENTS

| Number       | Name       | Date           |
|--------------|------------|----------------|
| 17,895       | Roth       | July 28, 1857  |
| 1,027,953    | Wickman    | May 28, 1912   |
| 1,645,061    | Kress      | Oct. 11, 1927  |
| 1,662,951    | Bragg      | Mar. 20, 1928  |
| 25 1,873,924 | Hirschkind | Aug. 23, 1932  |
| 2,071,308    | Hirschkind | Feb. 16, 1937  |
| 2,199,376    | Reichert   | Apr. 30, 1940  |
| 2,214,845    | Wells      | Sept. 17, 1940 |
| 2,290,601    | Reichert   | July 21, 1942  |
| 30 2,339,595 | Williams   | Jan. 18, 1944  |

#### FOREIGN PATENTS

| Number     | Country       | Date         |
|------------|---------------|--------------|
| 8,851      | Great Britain | A. D. 1904   |
| 35 442,336 | Great Britain | Feb. 6, 1936 |